# NEW EUROPEAN PATENT SPECIFICATION

(11) **EP 3 682 454 B2**
(45) Date of publication and mention of the opposition decision: **27.05.2026**
(45) Mention of the grant of the patent: 26.07.2023
(21) Application number: 18780233.5
(22) Date of filing: 07.09.2018
(51) Int. Cl.: G21G 1/10, H05H 6/00

(54) **METHOD FOR OBTAINING A SOLID TARGET FOR RADIOPHARMACEUTICALS PRODUCTION**
VERFAHREN ZUR GEWINNUNG EINES FESTEN ZIELS FÜR DIE HERSTELLUNG VON RADIOPHARMAZEUTIKA
PROCÉDÉ D'OBTENTION D'UNE CIBLE SOLIDE POUR LA PRODUCTION DE PRODUITS RADIOPHARMACEUTIQUES

(30) Priority: 14.09.2017 IT 201700102990
(43) Date of publication of application: 22.07.2020
(73) Proprietor: Istituto Nazionale di Fisica Nucleare, 00044 Frascati (RM) (IT)
(72) Inventor: PALMIERI, Vincenzo, 00044 Frascati (RM) (IT); SKLIAROVA, Hanna, 00044 Frascati (RM) (IT); CISTERNINO, Sara, 00044 Frascati (RM) (IT); MARENGO, Mario, 00044 Frascati (RM) (IT); CICORIA, Gianfranco, 00044 Frascati (RM) (IT)
(74) Representative: Metroconsult Srl
(86) International application number: PCT/IB2018/056826
(87) International publication number: WO 2019/053570

(56) References cited:
- WO-A2-02/099816
- US-A- 5 158 933
- US-A1- 2010 166 653
- US-A1- 2013 301 769
- QUEERN STACY LEE; AWEDA TOLULOPE ARAMIDE; MASSICANO ADRIANA VIDAL FERNANDES; CLANTON NICHOLAS ASHBY; EL SAYED RETTA; SADER JAYDEN : "Production of Zr-89 using sputtered yttrium coin targets89Zr using sputtered yttrium coin targets", NUCLEAR MEDICINE AND BIOLOGY, ELSEVIER, NY., US, vol. 50, 23 March 2017 (2017-03-23), US , pages 11 - 16, XP085047005, ISSN: 0969-8051, DOI: 10.1016/j.nucmedbio.2017.03.004

## Description

### BACKGROUND

The present invention relates to the field of radionuclides production and, in particular, to a method for obtaining a target or solid state target, for use in the production of radiopharmaceuticals for diagnostic and therapeutic purposes, through use of a particle accelerator, more particularly a cyclotron.

The present invention also relates to a system for production of said radionuclides.

### STATE OF THE ART

Nuclear Medicine is a branch of medicine that uses radiopharmaceuticals both for diagnostic and therapeutic purposes.

One of these, ^{99m}Tc, is an extremely important radioactive isotope, used in almost all types of traditional diagnostic exams.

^{99m}Tc is currently extracted from portable generators containing the precursor radioactive isotope ⁹⁹Mo coming from fission reactors, which use highly enriched ²³⁵U. As of today, 95% of ⁹⁹Mo is produced by five plants which are over 50 year old and, since the stable supply of ⁹⁹Mo cannot be guaranteed in the future, alternative routes for the production of ^{99m}Tc based on particle accelerators (cyclotrons) were developed.

Currently, the reaction ¹⁰⁰Mo(p,2n)^{99m}Tc is considered to be the most favourable for the direct production of ^{99m}Tc by means of a cyclotron, starting from the precursor isotope ¹⁰⁰Mo, and it was found that, in order to obtain the maximum production of ^{99m}Tc with minimal impurities by means of small medical cyclotrons (e.g., GE PETtrace supporting a standard current of about 100 mA), it is necessary to impart the protons in the cyclotron, intended to hit a target formed by a layer of enriched ¹⁰⁰Mo and having a thickness of the order of about 100 mm, applied to a corresponding supporting element (in technical jargon also backing), an energy optionally comprised between about 10 MeV and about 22 MeV.

In this regard, various targets for different types of cyclotron have been developed and tested and various irradiation tests with ¹⁰⁰Mo, metal oxide and carbide natural Mo, applied to different supporting elements [1, 2]have been conducted.

The radiopharmaceutical production requires that the targets to be used in combination with a cyclotron meet two fundamental requirements: they must guarantee a high level of heat dissipation, so as to be able to apply the maximum current that can be delivered by the cyclotron, during the irradiation of the target, and obtain the maximum production yield; and they must also ensure a high inertia of the supporting element in (standard) conditions of the target dissolution, to guarantee the chemical and radiochemical purity of the final product.

Although oxides [1-5], carbides [1, 2], and also targets in solution [1, 2] have been studied, metal Mo targets are considered the most suitable for the purpose, since the metal Mo target provide high production yields of ^{99m}Tc.

This is due to the high level of heat dissipation, associated with a good thermal conductivity of metal. In fact it was noted that just the presence of oxygen traces drastically reduces the thermal conductivity of the material.

For the production of a target having the above mentioned characteristics of heat dissipation and chemical inertia, two different approaches have been taken into consideration at present. According to a first approach, one target can be manufactures by means of a preparation step of a coin or pellet of precursor isotope of Mo, followed by a subsequent step of adhesion to a supporting element. According to a second approach, the precursor isotope of Mo is directly deposited on a supporting element.

With reference to the first approach, ¹⁰⁰Mo is commercially available in the form of metal powder, therefore different research groups have proposed the transformation of the powder of ¹⁰⁰Mo in a dense and not porous pellet or sheets - using different methods, including pressing, sintering and lamination - to be applied to a respective supporting element.

However, the targets produced only by hydraulic pressing of metal powder [1, 2, 6-8] have proven to be able to support only low cyclotron currents, because the density of the pellets thus produced is much less than that of the bulk material.

With the sintering technique of Mo powders [2, 9, 10] in reduced or inert atmosphere [1, 2, 6-8] followed by pressure bonding [1, 2, 6-8] or vacuum brazing [2, 9, 10] targets of Mo were made which support currents of the order of hundreds of mA and standard procedures are considered rolling, starting from dust or beads of Mo, produced by melting the powder through e-beam [1, 2, 11], or recasting of the Mo powders followed by remodelling through rolling.

The targets produced according to the first approach have shown, however, not to be fully satisfactory. In fact, they showed to be adequate for manufacturing, since it is very difficult to provide a good thermal contact between the pellets or sheets of Mo and the supporting element, during irradiation by the cyclotron.

With reference to the second approach for manufacturing a target for the production of ^{99m}Tc, direct deposition of Mo on a supporting element was obtained by direct fusion of the powders of Mo on the support material (backing) itself [12]. This approach, however, has shown that it does not guarantee an acceptable uniformity of the layer of Mo.

It has also been considered also the technique of electrodeposition of metals in aqueous solutions, which is a well known industrial process, but it has proved to be difficult to deposit refractory metals such as Mo, with standard techniques of electrodeposition, due to their great affinity with oxygen. Techniques have been disclosed of electrodeposition, in particular alkaline solutions [13] or acetates [14]. This type of deposition has shown a high level of oxidation and a thickness no greater than about 20 mm.

In addition, the electrodeposition process from aqueous solution is very inefficient. In fact, only a percentage quantity of Mo below 2% remains deposited onto the support material, due to the high affinity of Mo with the oxygen of the aqueous solution. Moreover, it has been reported [15] that the co-deposition of molybdenum with zinc is much more efficient. The electrodeposition in ionic liquids or molten salts [2, 16, 17] provides for a better quality of the layer of Mo, but requires expensive equipment and more difficult protocols.

With the electrophoretic deposition from a mixture of powders of Mo and additives, followed by sintering at high temperature, Mo films were obtained having a sufficient thickness, resistant to a current of 300 mA, at conditions of target inclined, at power density reduced with respect to an orthogonal target and same intensity of current delivered [1, 18]. Through further improvements to the sintering process in inert atmosphere [2] the actual targets support up to 500 mA.

The main disadvantage of all electrochemical deposition methods mentioned above is, however, the incapacity of avoiding impurities coming from the electrolytic bath in the manufactured target, which is a serious limit for medical applications relating to the present invention.

PVD methods of direct deposition of Mo have also been considered, which include a thermal spray (Thermal spray) [19], cathodic arc [2], argon [20] and xenon [21]sputtering FIB.

At the moment information regarding tests under cyclotron beam are not available for target obtained by the arc sputtering and FIB technique and, although with the FIB-sputtering technique thicknesses of Mo films more than a few microns have not been reported, the method seems very interesting because it allows: the use of minimum quantities of isotope, to have very low losses of the expensive material (enriched¹⁰⁰Mo ) during deposition, and to obtain a high purity of the target thus manufactured.

With reference to the supporting element to which enriched ¹⁰⁰Mo is to be directly applied or deposited for the production of ^{99m}Tc, at the moment the materials tested for its production are many and among them is copper [1, 2, 19, 22], aluminium [1, 2, 6-8, 11], the tantalum [1, 2, 6-8, 12, 18]GLIDCOP[2, 9, 10] and platinum [1, 2, 13].

The process of standard production of ^{99m}Tc with the reaction ¹⁰⁰Mo(p, 2n)^{99m}Tc, provides, as mentioned above, for the irradiation by a cyclotron of a target comprising enriched ¹⁰⁰Mo and, after such irradiation, a standard step of dissolution of Mo and of the mixture of Tc in H₂O₂ at a high temperature, optionally comprised between 60°C and 90°C. However, since the transition, post transition and refractory metals used up to now as support materials are not perfectly chemically inert under these conditions, even very small amounts of impurities in the mixture of Mo, Tc, H₂O₂ can compromise the production of the radiopharmaceutical.

Therefore, there is a continuing demand for innovation regarding the manufacturing of targets for the production of radiopharmaceuticals by use of particle accelerators, in particular for the production of ^{99m}Tc.

The need to develop a method for obtaining a target that can be used in the production of radiopharmaceuticals is therefore felt, in particular for the production of ^{99m}Tc, allowing to minimize or eliminate the above mentioned drawbacks.

Document US 2010/0166653 A1 discloses compositions of high specific activity SN-117M and methods of preparing the same.

### OBJECTS OF THE INVENTION

The main object of the present invention is to improve the state of the art in the field of production, through small sized particle accelerators (for example GE PETtrace), of radionuclides in general and ^{99m}Tc, in particular.

More particularly, it is an object of the present invention to provide for a method for obtaining a target, which target can be used in the production of a radionuclide, allowing for heat dissipation, during the irradiation step, which is higher with respect to traditional targets.

Another object of the present invention is to provide for a method for obtaining a target, which target can be used in the production of a radionuclide, allowing obtaining a high thickness and a high uniformity of the precursor isotope coupled to the respective supporting element, with respect to the traditional targets.

A further object of the present invention is to provide for a method for obtaining a target, which target can be used in the production of a radionuclide, allowing obtaining low oxidation levels and a high adhesion of the precursor isotope coupled to the respective supporting element, with respect to the traditional targets.

A further object of the present invention is to provide for a method for obtaining a target, which target can be used in the production of a radionuclide, allowing reducing impurities generated in the production process, with respect to the traditional targets.

A still further object of the present invention is to provide for a system for the production of a radiopharmaceutical, allowing optimizing the radiopharmaceutical production, with respect to the traditional systems.

These and further aspects of the present inventions will be obtained by a method for obtaining a target, which target can be used in the production of a radionuclide, according to claim 1.

The dependent claims refer to preferred and advantageous embodiments of the invention.

### BRIEF DESCRIPTION OF THE DRAWINGS

The present invention will be now described, for illustrative but not limiting purposes, according to its preferred embodiments, with particular reference to the drawings in the accompanying Figures, wherein:
Figure 1 shows a target which can be obtained by means of a preferred embodiment of the method of the present invention;
Figure 2 shows the main steps of the preferred embodiment of the method for obtaining the target of Figure 1;
Figure 3 shows process parameters relating to a step of the method of Figure 2;
Figure 4 illustrates the main elements of a system for dissolving the target of Figure 1;
Figure 5 is a scaled-up representation with parts in cross-section and in transparency, of some elements of the dissolution system of Figure 4; and
Figures 6a and 6b show some images relating to results of experimental tests conducted on a target obtained according to the method of the present invention.

### EMBODIMENTS OF THE INVENTION

Before going into the merits of the invention, it is of note that in the description and in the claims which follow, explicit reference is made and will be made to radioactive isotope ^{99m}Tc, but it is clear that the teachings of the present invention can be used for the production of other radioactive isotopes of medical interest, among which, purely by way of example, ⁶⁸Zn for the production of ^{64,67}Cu, radioactive isotopes ⁶⁸Ga, ⁸⁹Y or ^{nat}Y for the production of ⁸⁹Zr, ⁵²Cr for the production of ⁵²Mn, ^{nat}Ti for the production of ⁴⁸V, the ^{nat,63}Cu for the production of ^{62,63}Zn, etc. are mentioned.

It is also of note that the use of the terms "for example", "etc.", "or" indicates not exclusive alternatives without limitation, unless otherwise indicated, and the use of the term "includes" means "includes but is not limited to" unless otherwise indicated.

This being said, with reference to the accompanying drawings, it will be noted that a method for obtaining a solid target (represented in Figure 1 with reference numeral 1) for the production of at least one radionuclide by cyclotron, according to the present invention, is indicated with reference numeral 100 and comprises at least one first step (step 110) of providing at least one first supporting element 2, having at least one first surface 21, intended to support in use at least one precursor isotope 3, and at least one second surface 22 opposite to the first surface 21; and at least one second step (step 120) of application of said at least one precursor isotope 3 on the first surface 21.

The first supporting element 2 typically has a substantially flat configuration, for example circular or elliptical or rectangular in plan, with opposite surfaces 21 and 22 theirbetween, and can be obtained in bulk material, or in the form of layer, applicable, as will be explained hereinafter, to one second supporting element 4.

The first supporting element 2 is advantageously made of a chemically inert material (dielectric) under the conditions of dissolution of the precursor isotope 3 applied thereto and of the radioactive isotope produced after the irradiation by the cyclotron, in a deprived or not oxygen atmosphere), more in particular it is a material that is chemically inert with respect to a dissolution mixture with which it is intended to come into contact for further chemical separation between precursor isotope and radioactive isotope obtained, following the irradiation by the cyclotron.

In the specific case of production of radioactive isotope ^{99m}Tc produced starting from ¹⁰⁰Mo, the chemically inert material (dielectric) at the conditions of dissolution, which makes up the first supporting element 2, comprises a material chosen among sapphire, synthetic diamond, quartz, glass, silicon, carbon compounds, glassy carbon, silicon oxide, aluminium oxide, magnesium oxide, zirconium oxide, advanced ceramics, or DLC (Diamond-like carbon or synthetic diamond), graphene, polymeric materials and the like or combinations thereof. The first supporting element 2 can also be made of copper or copper and diamond or copper electrodeposited on a goretex net, with the first surface 21, intended to support at least one precursor isotope 3, gold covered by sputtering or galvanic plating.

With reference to step 120 of the method according to the present invention, of application of at least one precursor isotope 3 on the first surface 21 of the first supporting element 2, it comprises at least one step of magnetron sputtering of said at least one precursor isotope 3 on the first surface 21, allowing to obtain one film of precursor isotope 3 having a high density level.

In this regard, preliminary tests have demonstrated that with said magnetron sputtering technique, it is possible to obtain a film of precursor isotope 3 having a density greater than 98% of bulk density, while with pressing and sintering techniques density ranging between 80% and 95% (the maximum density is obtained at particularly specific sintering conditions in a reducing atmosphere) are obtained, and with other conventional techniques, the density of the in the precursor isotope 3 film is the following:
- with pressing, less than 80% of bulk density,
- with electrode position, less than 80% of bulk density; and
- with electrophoresis, comprised between 40% and 60% of bulk density.

Moreover, thanks to the magnetron sputtering technique, a film of precursor isotope 3 having uniformity, thickness and adhesion to the first supporting element 2 is obtained.

In this respect, the method of the present invention comprises one step 125 of setting the process parameters for said step 120, so that, in said deposition step, the total stress of the system, composed by the first supporting element 2 and the film by precursor isotope 3, is minimized.

The total stress of the system, as is well known, is given by the residual stress (intrinsic) of the film of precursor isotope 3 applied to the first supporting element 2, and by the stress associated with the thermal discrepancy (in technical jargon also thermal mismatch or σ_{mismatch}) between the film of isotope precursor 3 and the first supporting element 2.

The use of the magnetron sputtering technique is particularly advantageous in the present invention, because it can be used for direct deposition of isotopes on fragile - i.e. inclined to break, if subjected to an external force, with no deformation or stretching occurring beforehand - first supporting elements, i.e. the dielectric, ceramic, non-metallic materials mentioned above, including: DLC, quartz, sapphire, etc.

The intrinsic stress (σ_{intrinsic}) in the deposited films depends, as is known, by the energy supplied to the surface of the precursor isotope 3 film, increasing thickness during the deposition. The variables significantly involved in the change of energy and, therefore, in the mechanism for the growth of the thickness of said film, are the sputtering gas, the temperature of the sample stage, the bias (i.e. a potential applied to sample holder), etc. Theoretically there is one sputtering gas pressure marking the passage from the traction to the compression stress. At relatively high pressures, the frequency of collisions between the atoms of the gaseous phase increases, reducing the kinetic energy of the sputtered atoms and of reflected neutral atoms bombarding the film of precursor isotope 3 during its thickness growth, thereby providing a porous microstructure; the interatomic attraction forces between the edges of the grain, therefore produce a traction stress. At low pressures, the atoms of the precursor isotope 3 that are deposited on the first supporting element 2 have a high kinetic energy and the resulting film of precursor isotope 3 has a dense microstructure, promoting compression stress. The temperature of the substrate influences, moreover, the kinetic energy of the particles of precursor isotope 3 already deposited on the first supporting element 2. A low temperature, which depends on the material, the pressure and that, according to the Structure Zone Model is given by Tₕ<0.2 with T_{H}=T_{depos}/Tₘₑₗₜ (in Kelvin) where T_{depos} is the temperature of the substrate (sample carrier) during the process and Tₘₑₗₜ is the melting temperature of the material to be deposited, promotes, in fact, a microstructure of columnar type with microscopic voids, associated with a traction stress. A high temperature, which always depends on the material and the pressure and that, according to the Structure Zone Model is given by Tₕ>0.3, corresponds to an increase in the mobility of the atoms of the precursor isotope 3, which leads to a structure of type bulk and a negligible "thermally induced" stress.

According to a particularly advantageous aspect of the method of the present invention, the step 120 of applying the precursor isotope 3 on said first supporting element 2 comprises a multilayer deposition of said at least one precursor isotope 3, and between a deposition step and the next at least one relaxation time period is optionally provided for, optionally comprised between a few milliseconds to a few hours, during which the layer of precursor isotope 3 applied to the first supporting element 2 is hardening.

With reference to the aforementioned second component of the total stress of the system, i.e. the stress due to thermal mismatch (σ_{mismatch}) between precursor isotope 3 and first supporting element 2, it is detected, in general, in structures having very different coefficients of thermal expansion, subject to a uniform change of temperature. When a film of precursor isotope 3 is deposited on one first supporting element, usually at high temperature, i.e. Tₕ> 0.3 as defined above and, in the case of Mo, higher than 500°C, and is subsequently cooled and brought to room temperature, the difference between the coefficients of thermal expansion between the film of precursor isotope 3 and the first supporting element 2 determines the generation of a stress. If the coefficient of thermal expansion of the film of precursor isotope 3 is smaller than that of the first supporting element 2, a compressive stress will result or, vice versa, a traction stress.

This being said, since the coefficients of thermal expansion which cause the stress due to the mismatch σ_{mismatch}, vary in function of the material used for the first supporting element 2, the intrinsic stress of the film of precursor isotope σ_{intrinsic} is adapted to minimise the total stress of the system (σₜₒₜ= σ_{mismatch}+σ_{intrinsic}), in the method of the present invention.

Purely by way of example and with reference to obtaining a target for the production of ^{99m}Tc, starting from ¹⁰⁰Mo, the process parameters set at step 125 of the method according to the present invention, for the application, by magnetron sputtering, of a layer of ¹⁰⁰Mo having a thickness of about 110 mm on a substrate of sapphire (0̸ 13 mm x 0.5 mm, quality IR, with optical finish) and wherein the total stress of the system is minimized, are reported below.

The film of ¹⁰⁰Mo was deposited by DC magnetron sputtering with a source of planar cathode (2 inches). The deposition was performed on a planar sample holder, heated to 500°C, 6 cm away from the cathode. The optimized sputtering parameters are shown in Table 1 (Figure 3 attached). Experimental tests have demonstrated that the film of Mo deposited with this technique of magnetron sputtering, under conditions shown in Table 1, advantageously possesses the same density of the bulk material, good adhesion to the substrate, greater than 98% of bulk density, and no signs of oxidation.

The method for obtaining a solid target, usable in the production of at least one radionuclide, according to the present invention, comprises a further step (step 130) of coupling between said at least one first supporting element 2 and at least one second supporting element 4, at the second surface 22 of the first supporting element 2, said at least one second supporting element 4 comprising at least one material having a high thermal conductivity and mechanical stability, even chemically not inert at the conditions of dissolution of the precursor isotope 3 and of the radioactive isotope produced as a result of irradiation, by a cyclotron.

Such a second supporting element 4 can be made of a material selected between copper, silver, aluminium and/or their compounds.

The coupling between the first and second supporting element (2, 4) allows compensating, in part, the low thermal conductivity, for example less than 50W/(mK), of the first supporting element 2 made of dielectric material and obtaining, therefore, for target 1 thereby manufactured, higher levels of heat dissipation during the irradiation of the same, by the cyclotron. By way of example, consider in fact that the thermal conductivity of the sapphire is approximately equal to 40W/(mK) and that of quartz is equal to about 8W/(mk).

The second supporting element 4 has a flat shape, and delimits a seat 41, suitably configured and provided for coupling with the second surface 22 of the first supporting element.

The second supporting element 4 may have any configuration, provided it is suitable for insertion in a respective housing seat of the cyclotron used for the production of the radionuclide.

According to the present invention, this step 130 of coupling between the first supporting element 2 and the second supporting element 4 comprises at least one step of vacuum brazing between the first supporting element 2 and at least the second supporting element 4.

This vacuum brazing step is particularly advantageous for the present invention since it allows obtaining a high thermal and mechanical stability between the first and the second supporting element.

The brazing step 130 occurs, alternatively, in an inert atmosphere and this helps to prevent oxidation of the metal part and the brazing material used and, therefore, it guarantees a better thermal contact between the two supporting elements 2 and 4.

The person skilled in the art will have no difficulty in understanding that the brazing material, selected for use in step 130 of the method according to the present invention, will be different depending on the materials of which the first and the second supporting element are made and will be selected in such a way as to reduce to the minimum the stress due to thermal mismatch (σ_{mismatch}) generated during the brazing process.

According to a background example not belonging to the present invention, step 130 of coupling, between the first supporting element 2 and the second supporting element 4, comprises the direct deposition of the first supporting element 2 on at least the second supporting element 4 and in particular, the direct deposition of any one of the materials mentioned above for the first supporting element 2 (among which, DLC, aluminium oxide, zirconium oxide, silicon oxide, etc.) on the second supporting element 4 having a high conductivity, by means of appropriate methods such as CVD, PECVD, reactive sputtering.

Optionally, the method according to the present invention further comprises a metallization step (step 115) of at least one second surface 22 of the first supporting element 2, before the coupling step between the second surface and the second supporting element 4 and, optionally, before step 120 of deposition of the film of precursor isotope 3 on the supporting element.

The metallization is carried out according to known metallization techniques, for example through chemical, electrochemical deposition, PVD deposition, mechanical deposition, etc., using appropriate metals, such as Ti or Ni.

Purely by way of example and with reference to obtaining a target for the production of ^{99m}Tc, starting from the precursor isotope of ¹⁰⁰Mo, a target comprising both the first supporting element 2 and the second supporting element 4, coupled by means of vacuum brazing was obtained and composed as follows:
- the first supporting element is made of sapphire (0̸ 13 mm x 0.5 mm, quality IR, optical finish) or synthetic diamond (0̸ 13.5 mm x 0.4 mm, with thermal conductivity 1500W/(mK);
- the second supporting element is made of copper (0̸ 32 mm x 1 mm) having high thermal conductivity; the brazing material used is a paste of Cu-Ag-Ti, obtained by mixing the powder of the corresponding elements with a binder, the Coccoina i.e. a glue of partially hydrolysed potato starch, and water. By way of example, the percentages of the various components of the brazing material can be the following: metal powder 82%, Coccoina, 7.3% and water 10.7% by weight, with the metal powder thus composed: Cu 35.3 % - Ag 63 % - Ti 1.7 % by weight;
- the second surface 22 of the first supporting element 2 in sapphire or synthetic diamond, destined to come into contact with the second supporting element 4, has previously been metallised with a layer of approximately 1 mm of Ti, deposited by magnetron sputtering.

The brazing process was carried out in vacuum, at 950°C, maintaining a heating rate of 3°C/min and cooling rate of 2°C/min, to minimize thermomechanical stress in the final target.

This being said, the above described method allows to obtain one target that achieves the objects mentioned above, since it allows a high heat dissipation during the irradiation step, has a high thickness and high uniformity of the precursor isotope 3 coupled to the respective supporting element by magnetron sputtering, low levels of oxidation and a high adhesion of the precursor isotope coupled to the respective first supporting element.

It is advantageously usable in a dissolution system, which also forms the object of the present invention, of at least one precursor isotope 3 and at least one radioactive isotope produced as a result of irradiation by cyclotron - shown, in particular, in Figures 4 and 5.

Such a dissolution system is indicated in the figures by reference 200 and comprises:
- at least one target 1, obtained as described above, and
- at least one vial 210, intended to come into contact with the target 1 and defining with it at least one containment cavity 220, for at least one dissolution solution of the precursor isotope 3 and of the produced radioactive isotope, included in the target 1, as a result of irradiation by cyclotron.

Advantageously, the vial 210, for example made of PEEK, and the target 1 are mutually configured in such a way that the containment cavity 220 remains, in use, delimited between the vial 210 and the first supporting element 2 of the target 1, which is chemically inert under the conditions of dissolution of the precursor isotope 3 and the radioactive isotope produced as a result of irradiation, so that a dissolving solution for that precursor isotope 3 and for its products never comes into contact with the second supporting element 4, during the dissolution step of the target.

In the specific case of obtaining of a solid target for the production of ^{99m}Tc, starting from ¹⁰⁰Mo, the standard dissolution procedure of the target after irradiation provides for the dissolution of the isotope ¹⁰⁰Mo and the radioactive isotope produced ^{99m}Tc, in a solution of concentrated H₂O₂, for further chemical separation.

In these conditions of dissolution, the second supporting element 4, for example made of copper, would release chemical contamination which would compromise the effectiveness of the method of production of the radioactive isotope ^{99m}Tc.

The system described above, instead, avoiding contact between the dissolution solution and the second supporting element 4 of the target 1, chemically not inert with respect thereto, allows obtaining a produced radioactive isotope ^{99m}Tc of high purity.

As a demonstration of the effectiveness of the method and system described above, results of experimental tests conducted under the conditions set out below are reported.

A solid target 1 obtained by the method of the present invention and comprising a film of thickness equal to 110 mm of precursor isotope ^{nat}Mo deposited by magnetron sputtering on a first supporting element 2 in sapphire or synthetic diamond, vacuum brazed according to the method explained above, and with the second supporting element 4 made of copper with a high thermal conductivity, was tested subjected to a proton beam with energy of 16 MeV, using a cyclotron GE PETtrace.

The target 1 showed an excellent mechanical stability during the irradiation up to 60 mA current.

Experimental tests conducted, inter alia, on a target 1 composed of a layer of Mo having a thickness of 110 mm, applied by sputtering to a first supporting element 2 in sapphire, having diameter of 12.7 mm and thickness of 0.5 mm, in turn brazed on a second supporting element 4 made of copper, have shown a high mechanical stability (absence of cracks or other deformations of the target) at irradiation conditions at the maximum deliverable energy (15.6MeV), for 1 min, at 30 mA, 40 mA and 60mA (Figure 6a).

Excellent mechanical stability has been verified experimentally also on targets 1 having the same characteristics indicated above but one layer of Mo of greater thickness, equal to about 125 mm.

Experimental tests were also conducted also on a target 1 composed of a layer of Mo having a thickness of 125 mm, applied by sputtering to a first supporting element 2 made of synthetic diamond, having diameter of 13 mm and a thickness of 0.3 mm, in turn brazed on a second supporting element 4 made of copper. The tests results demonstrated a high mechanical stability (absence of cracks or other deformations of the target) at irradiation conditions at the maximum deliverable energy (15.6MeV), for 1 min, at 30 mA, 40 mA and 60mA (Figure 6b).

Excellent mechanical stability has been verified experimentally even on one target 1 having the same characteristics but at conditions closer to working conditions. The irradiation of the cyclotron lasted for 30 min at 60mA and at 15.6 MeV of energy delivered. The target 1 has demonstrated excellent resistance without any sign of mechanical damage.

The dissolution of the irradiated material was carried out in a vial in 1 ml of H₂O₂ at 30% by weight, 70°C and 10ml of this solution was analysed with a gamma spectrometer of the Research Laboratory of the Department of Medical Physics of the Sant'Orsola Hospital of Bologna.

Between the radioactive isotopes identified with the gamma spectrometry only products of the irradiation of the natural Mo were present: ^{92m}Nb, ⁹⁴Tc, ^{95m}Tc, ⁹⁶Tc, ⁹⁹Mo, ^{99m}Tc.

The chemical inertia, in particular, of the sapphire and synthetic diamond was proven because no contaminant was present in the solution, and especially the effectiveness of the solid target obtained according to the method of the present invention.

In the foregoing the preferred embodiments were described and some modifications of this invention have been suggested, but it should be understood that those skilled in the art can make modifications and changes without departing from the relative scope of protection, as defined by the appended claims.

### Bibliographical references

[1] Report on the 2nd Research Coordination Meeting on "Accelerator-based Alternatives to Non-HEU Production of 99Mo/99mTc", 7-11 October 2013, in, Legnaro, Italy, 2013.
[2] Report on the 3nd Research Coordination Meeting on "Accelerator-based Alternatives to Non-HEU Production of 99Mo/99mTc", June 22-26, 2015, in, Vienna, Austria, 2015.
[3] K. Nishikata, A. Kimura, T. Ishida, S. Kitagishi, K. Tsuchiya, H. Akiyama, M. Nagakura, K. Suzuki, Method of producing radioactive molybdenum, (2013).
[4] A. Avetisyan, R. Dallakyan, R. Sargsyan, A. Melkonyan, M. Mkrtchyan, G. Harutyunyan, N. Dobrovolsky, The powdered molybdenum target preparation technology for 99mTc production on C18 cyclotron, International Journal of engineering and Innovative Technology, 4 (2015) 37-44.
[5] L.A.M.M. Barbosa, System and method for producing radiomedical-grade tc-99m, (2014).
[6] K. Gagnon, J.S. Wilson, C.M.B. Holt, D.N. Abrams, A.J.B. McEwan, D. Mitlin, S.A. McQuarrie, Cyclotron production of 99mTc: Recycling of enriched 100Mo metal targets, Appl. Radiat. Isot., 70 (2012) 1685-1690.
[7] K. Gagnon, S. McQuarrie, J. Wilson, Production of technetium from a molybdenum metal target. Patent WO 2012139220 A1, in, The Governors Of The University Of Alberta, United States, 2012.
[8] J. Wilson, K. Gagnon, S. McQuarrie, Production of technetium from a molybdenum metal target, in, The governors of University of Alberta, United States, 2014.
[9] S.K. Zeisler, V. Hanemaayer, K.R. Buckley, Target system for irradiation of molybdenum with particle beams. Patent WO2015161385 A1, in, Triumf, United States, 2015.
[10] P. Schaffer, F. Bénard, A. Bernstein, K. Buckley, A. Celler, N. Cockburn, J. Corsaut, M. Dodd, C. Economou, T. Eriksson, Direct Production of 99m Tc via 100 Mo (p, 2n) on Small Medical Cyclotrons, Physics Procedia, 66 (2015) 383-395.
[11] S. Manenti, U. Holzwarth, M. Loriggiola, L. Gini, J. Esposito, F. Groppi, F. Simonelli, The excitation functions of 100 Mo (p, x) 99 Mo and 100 Mo (p, 2n) 99m Tc, Appl. Radiat. Isot., 94 (2014) 344-348.
[12] A. Zyuzin, B. Guérin, E. van Lier, S. Tremblay, S. Rodrigue, J.A. Rousseau, V. Dumulon-Perreault, R. Lecomte, J.E. van Lier, Cyclotron Production of 99mTc, in: WTTC, 2012.
[13] C.G. Fink, Electroplating and process of producing same. Patent 1,885,700, in, 1932.
[14] T.J. Morley, L. Penner, P. Schaffer, T.J. Ruth, F. Bénard, E. Asselin, The deposition of smooth metallic molybdenum from aqueous electrolytes containing molybdate ions, Electrochem. Commun., 15 (2012) 78-80.
[15] H. Kazimierczak, P. Ozga, R.P. Socha, Investigation of electrochemical co-deposition of zinc and molybdenum from citrate solutions, Electrochim. Acta, 104 (2013) 378-390.
[16] G.J. Kipouros, D.R. Sadoway, The electrodeposition of improved molybdenum coatings from molten salts by the use of electrolyte additives, J. Appl. Electrochem., 18 (1988) 823-830.
[17] N. Ene, C. Donath, Texture of electrolytic Mo deposition from molten alkali halide, Journal of Optoelectronics and Advanced Materials, 8 (2006) 708.
[18] P. Schaffer, F. Benard, K.R. Buckley, V. Hanemaayer, C.H. Manuela, J.A. Klug, M.S. Kovacs, T.J. Morley, T.J. Ruth, J. Valliant, Processes, systems, and apparatus for cyclotron production of technetium-99m. Patent US 2013/0301769 A1, in, TRIUMF, United States, 2013.
[19] A.R. Jalilian, H. Targholizadeh, G.R. Raisali, H. Zandi, M.K. Dehgan, Direct Technetium radiopharmaceuticals production using a 30MeV Cyclotron, DARU: Journal of Faculty of Pharmacy, Tehran University of Medical Sciences, 19 (2011) 187.
[20] H. Folger, J. Klemm, M. Muller, Preparation of Nuclear Accelerator Targets by Focused Ion Beam Sputter Deposition, Nuclear Science, IEEE Transactions on, 30 (1983) 1568-1572.
[21] P.S. Morrall, The Target Preparation Laboratory at Daresbury, Nuclear Instruments and Methods in Physics Research Section A: Accelerators, Spectrometers, Detectors and Associated Equipment, 590 (2008) 118-121.
[22] H.J. Maier, H.U. Friebel, D. Frischke, R. Grossmann, State of the art of high vacuum sputter deposition of nuclear accelerator targets, Nuclear Instruments and Methods in Physics Research Section A: Accelerators, Spectrometers, Detectors and Associated Equipment, 334 (1993) 137-141.

## Claims

1. Method for obtaining a solid target for radionuclides production by cyclotron, comprising the steps of:
- arranging at least one first supporting element (2), having at least one first surface (21) intended to support at least one precursor isotope (3) - (step 110);
- applying said at least one precursor isotope (3) on said at least one first surface (21) of said at least one first supporting element (2) - (step 120);
said at least one first supporting element (2) being a chemically inert material at conditions of dissolution of said at least one precursor isotope (3) and at least one radioactive isotope of interest produced upon irradiation of said target (1) by said cyclotron;
said step (120) of applying said at least one precursor isotope (3) on said at least one first surface (21) of said at least one first supporting element (2) comprising at least one magnetron sputtering step of said precursor isotope (3) on at least one said first surface (21),
**characterized by** the fact that
the method further comprises the step (130) of coupling between said at least one first supporting element (2) and at least one second supporting element (4), in correspondence of at least one second surface (22) of said at least one first supporting element (2) opposite to said at least one first surface (21), said at least one second supporting element (4) comprising at least one material having high thermal conductivity and mechanical stability, and being chemically non inert at conditions of dissolution of said at least one precursor isotope (3) and at least one radioactive isotope of interest produced on said at least one first supporting element (2) upon irradiation by said cyclotron, said material of said at least one second supporting element (4) being optionally selectable out of copper, silver, aluminium and/or their compounds,
wherein said step (130) of applying said at least one first supporting element (2) on said at least one second supporting element (4), comprises at least one step of brazing in vacuum or inert gas, between said at least one first supporting element (2) and said at least one second supporting element (4).

2. Method according to claim 1, wherein said magnetron sputtering step comprises at least one multi-layer deposition step of said at least one precursor isotope (3), on said at least one first supporting element (2), providing at least one relaxation time between a deposition step and the next one, optionally ranging from few milliseconds up to few hours.

3. Method according to any one of the preceding claims, wherein said magnetron sputtering step comprises at least one preliminary step (125) of process parameter setting, such that during said magnetron sputtering step the total stress of a system, comprising said at least one first supporting element (2) and said at least one radioactive precursor isotope (3), is minimized, said total stress of the system comprising the intrinsic residual stress of said at least one precursor isotope (3) applied to said at least one first element (2) and the stress associated with the thermal mismatch between said at least one first supporting element (2) and said at least one precursor isotope (3).

4. Method according to any one of the preceding claims, wherein said at least one first supporting element (2) comprises a non-metallic material in a layer form, applicable on at least one second supporting element (4).

5. Method according to any one of the preceding claims, wherein said at least one first supporting element (2) is made of a dielectric material selected out of sapphire, synthetic diamond, quartz, glass, silicon, carbon compounds, glassy carbon, silicon oxide, aluminium oxide, magnesium oxide, zirconium oxide, advanced ceramics, or DLC, graphene, polymers and the like.

6. Method according to any one of claims 1 to 3, wherein said at least one first supporting element (2) is made of copper or copper and diamond or copper electrodeposited on a goretex net, with said at least one first surface (21) gold covered by sputtering or galvanic plating.

7. Method according to any one of the preceding claims, comprising one step (115) of plating at least said second surface (22) of said at least one first supporting element (2), before said step (130) of applying said at least one first supporting element (2) on said at least one second supporting element (4) and optionally before said step (120) of applying said precursor isotope (3) on said supporting element.

8. Method according to any one of the preceding claims, wherein said step (130) of applying said at least one first supporting element (2) on said at least one second supporting element (4), comprises at least one step of direct depositing said at least one first supporting element (2) on said at least one second supporting member (4) by a technique selected out of CVD, PECVD or reactive sputtering.

## Patentansprüche

1. Verfahren zum Erhalten eines festen Targets zur Radionuklidproduktion durch ein Zyklotron, umfassend die Schritte:
- Anordnen mindestens eines ersten Tragerelements (2), das mindestens eine erste Oberflache (21) aufweist, die dazu bestimmt ist, mindestens ein Vorlauferisotop (3) zu tragen (Schritt 110);
- Aufbringen des mindestens einen Vorlauferisotops (3) auf die mindestens eine erste Oberflache (21) des mindestens einen ersten Tragerelements (2) (Schritt 120);
wobei das mindestens eine erste Tragerelement (2) ein Material ist, das unter Auflosungsbedingungen des mindestens einen Vorlauferisotops (3) und mindestens eines interessierenden radioaktiven Isotops, das bei Bestrahlung des Targets (1) durch das Zyklotron erzeugt wird, chemisch inert ist;
wobei der Schritt (120) des Aufbringens des mindestens emen Vorlauferisotops (3) auf die mindestens eine erste Oberflache (21) des mindestens einen ersten Tragerelements (2) mindestens einen Magnetron-Sputterschritt des Vorlauferisotops (3) auf mindestens eine erste Oberflache (21) umfasst,
**dadurch gekennzeichnet, dass**
das Verfahren den Schritt (130) des Koppelns zwischen dem mindestens einen ersten Tragerelement (2) und mindestens einem zweiten Tragerelement (4) in Übereinstimmung mit mindestens einer zweiten Oberflache (22) des mindestens einen ersten Tragerelements (2) gegenüber der mindestens einen ersten Oberflache (21) umfasst, wobei das mindestens eine zweite Tragerelement **(4)** mindestens ein Material umfasst, das eine hohe Warmeleitfühigkeit und mechanische Stabilitat aufweist und unter Auflosungsbedingungen des mindestens einen Vorlauferisotops (3) und mindestens eines interessierenden radioaktiven Isotops, das auf dem mindestens einen ersten Tragerelement (2) bei Bestrahlung durch das Zyklotron erzeugt wird, chemisch nicht inert ist, wobei das Material des mindestens einen zweiten Tragerelements **(4)** optional aus Kupfer, Silber, Aluminium und/oder deren Verbindungen ausgewahlt werden kann,
wobei der Schritt (130) des Aufbringens des mindestens einen ersten Tragerelements (2) auf das mindestens eine zweite Tragerelement **(4)** mindestens einen Schritt des Lotens in Vakuum oder Inertgas zwischen dem mindestens einen ersten Tragerelement (2) und dem mindestens einen zweiten Tragerelement **(4)** umfasst.

2. Verfahren nach Anspruch **1,** wobei der Magnetron-Sputterschritt mindestens einen mehrschichtigen Abscheidungsschritt des mindestens einen Vorlauferisotops (3) auf dem mindestens einen ersten Tragerelement (2) umfasst, der mindestens eine Relaxationszeit zwischen einem Abscheidungsschritt und dem nachsten bereitstellt, die optional von einigen Millisekunden bis zu einigen Stunden reicht.

3. Verfahren nach einem der vorhergehenden Ansprüche, wobei der Magnetron-Sputterschritt mindestens einen vorlaufigen Schritt (125) der Prozessparametereinstellung umfasst, so dass wahrend des Magnetron-Sputterschritts die Gesamtbelastung eines Systems, das das mindestens eine erste Tragerelement (2) und das mindestens eine radioaktive Vorlauferisotop (3) umfasst, minimiert wird, wobei die Gesamtbelastung des Systems die intrinsische Restbelastung des mindestens einen Vorlauferisotops (3), die auf das mindestens eine erste Element (2) aufgebracht wird, und die Belastung, die mit der thermischen Fehlanpassung zwischen dem mindestens einen ersten Tragerelement (2) und dem mindestens einen Vorlauferisotop (3) verbunden ist, umfasst.

4. Verfahren nach einem der vorhergehenden Ansprüche, wobei das mindestens eine erste Tragerelement (2) ein nichtmetallisches Material in Schichtform umfasst, das auf mindestens ein zweites Tragerelement **(4)** aufgebracht werden kann.

5. Verfahren nach einem der vorhergehenden Ansprüche, wobei das mindestens eine erste Tragerelement (2) aus einem dielektrischen Material hergestellt ist, das aus Saphir, synthetischem Diamant, Quarz, Glas, Silizium, Kohlenstoffverbindungen, glasartigem Kohlenstoff, Siliziumoxid, Aluminiumoxid, Magnesiumoxid, Zirkoniumoxid, fortgeschrittenen Keramiken oder DLC, Graphen, Polymeren und dergleichen ausgewahlt ist.

6. Verfahren nach einem der Ansprüche **1** bis 3, wobei das mindestens eine erste Tragerelement (2) aus Kupfer oder Kupfer und Diamant oder Kupfer hergestellt ist, das auf einem Goretex-Netz galvanisch abgeschieden ist, wobei die mindestens eine erste Oberflache (21) mit Gold durch Sputtern oder galvanisches Plattieren bedeckt ist.

7. Verfahren nach einem der vorhergehenden Ansprüche, umfassend einen Schritt (115) des Plattierens mindestens der zweiten Oberflache (22) des mindestens einen ersten Tragerelements (2) vor dem Schritt (130) des Aufbringens des mindestens einen ersten Tragerelements (2) auf das mindestens eine zweite Tragerelement **(4)** und optional vor dem Schritt (120) des Aufbringens des Vorlauferisotops (3) auf das Tragerelement.

8. Verfahren nach einem der vorhergehenden Ansprüche, wobei der Schritt (130) des Aufbringens des mindestens einen ersten Tragerelements (2) auf das mindestens eine zweite Tragerelement **(4)** mindestens einen Schritt des direkten Abscheidens des mindestens einen ersten Tragerelements (2) auf dem mindestens einen zweiten Tragerelement **(4)** durch eine Technik umfasst, die aus CVD, PECVD oder reaktivem Sputtern ausgewahlt ist.

## Revendications

1. Procédé d'obtention d'une cible solide pour la production de radionucléides par cyclotron, comprenant les étapes de :
- agencement d'au moins un premier élément de support (2), ayant au moins une première surface (21) destinée à supporter au moins un isotope précurseur (3) - (étape 110) ;
- application dudit au moins un isotope précurseur (3) sur ladite au moins une première surface (21) dudit au moins un premier élément de support (2) - (étape 120) ;
ledit au moins un premier élément de support (2) étant un matériau chimiquement inerte dans des conditions de dissolution dudit au moins un isotope précurseur (3) et d'au moins un isotope radioactif d'intérêt produit lors de l'irradiation de ladite cible (1) par ledit cyclotron ;
ladite étape (120) d'application dudit au moins un isotope précurseur (3) sur ladite au moins une première surface (21) dudit au moins un premier élément de support (2) comprenant au moins une étape de pulvérisation magnétron dudit isotope précurseur (3) sur au moins ladite première surface (21),
**caractérisé par le fait que**
le procédé comprend en outre l'étape (130) de couplage entre ledit au moins un premier élément de support (2) et au moins un deuxième élément de support (4), en correspondance d'au moins une deuxième surface (22) dudit au moins un premier élément de support (2) opposée à ladite au moins une première surface (21), ledit au moins un deuxième élément de support (4) comprenant au moins un matériau ayant une conductivité thermique et une stabilité mécanique élevées, et étant chimiquement non inerte dans des conditions de dissolution dudit au moins un isotope précurseur (3) et d'au moins un isotope radioactif d'intérêt produit sur ledit au moins un premier élément de support (2) lors de l'irradiation par ledit cyclotron, ledit matériau dudit au moins un deuxième élément de support (4) pouvant éventuellement être sélectionné parmi le cuivre, l'argent, l'aluminium et/ou leurs composés,
dans lequel ladite étape (130) d'application dudit au moins un premier élément de support (2) sur ledit au moins un deuxième élément de support (4), comprend au moins une étape de brasage sous vide ou sous gaz inerte, entre ledit au moins un premier élément de support (2) et ledit au moins un deuxième élément de support (4).

2. Procédé selon la revendication 1, dans lequel ladite étape de pulvérisation magnétron comprend au moins une étape de dépôt multicouche dudit au moins un isotope précurseur (3), sur ledit au moins un premier élément de support (2), assurant au moins un temps de relaxation entre une étape de dépôt et l'étape suivante, pouvant aller éventuellement de quelques millisecondes à quelques heures.

3. Procédé selon l'une quelconque des revendications précédentes, dans lequel ladite étape de pulvérisation magnétron comprend au moins une étape préliminaire (125) de définition de paramètres de procédé, de sorte que pendant ladite étape de pulvérisation magnétron la contrainte totale d'un système, comprenant ledit au moins un premier élément de support (2) et ledit au moins un isotope précurseur radioactif (3), soit minimisée, ladite contrainte totale du système comprenant la contrainte résiduelle intrinsèque dudit au moins un isotope précurseur (3) appliquée audit au moins un premier élément (2) et la contrainte associée à la disparité thermique entre ledit au moins un premier élément de support (2) et ledit au moins un isotope précurseur (3).

4. Procédé selon l'une quelconque des revendications précédentes, dans lequel ledit au moins un premier élément de support (2) comprend un matériau non métallique sous forme de couche, applicable sur au moins un deuxième élément de support (4).

5. Procédé selon l'une quelconque des revendications précédentes, dans lequel ledit au moins un premier élément de support (2) est réalisé en un matériau diélectrique sélectionné parmi le saphir, le diamant synthétique, le quartz, le verre, le silicium, des composés carbonés, le carbone vitreux, un oxyde de silicium, un oxyde d'aluminium, un oxyde de magnésium, un oxyde de zirconium, des céramiques techniques, ou le carbone sous forme de diamant amorphe DLC, le graphène, des polymères et autres analogues.

6. Procédé selon l'une quelconque des revendications 1 à 3, dans lequel ledit au moins un premier élément de support (2) est réalisé en cuivre et diamant ou cuivre électrodéposé sur un filet de type goretex, ladite au moins une première surface (21) étant recouverte d'or par pulvérisation ou placage galvanique.

7. Procédé selon l'une quelconque des revendications précédentes, comprenant une étape (115) de placage d'au moins ladite deuxième surface (22) dudit au moins un premier élément de support (2), avant ladite étape (130) d'application dudit au moins un premier élément de support (2) sur ledit au moins un second élément de support (4) et éventuellement avant ladite étape (120) d'application dudit isotope précurseur (3) sur ledit élément de support.

8. Procédé selon l'une quelconque des revendications précédentes, dans lequel ladite étape (130) d'application dudit au moins un premier élément de support (2) sur ledit au moins un deuxième élément de support (4), comprend au moins une étape de dépôt direct dudit au moins un premier élément de support (2) sur ledit au moins un deuxième élément de support (4) par une technique sélectionnée parmi le dépôt chimique en phase vapeur CVD, le dépôt chimique en phase vapeur assisté par plasma PECVD ou la pulvérisation réactive.
